

# UNITED STATES PATENT OFFICE.

RUDOLF RUTH AND ALADAR SCHULLER, OF OUDE-GOD, NEAR ANTWERP, BELGIUM.

## POLYCHROME SCREEN AND PROCESS OF MAKING THE SAME.

1,091,443.

Specification of Letters Patent. Patented Mar. 24, 1914.

No Drawing.

Application filed October 8, 1912. Serial No. 724,578.

To all whom it may concern:

Be it known that we, RUDOLF RUTH, a citizen of the United States of America, and ALADAR SCHULLER, a subject of the Emperor of Austria-Hungary, both residing at Oude-God, near Antwerp, Belgium, have invented certain new and useful Improvements in Polychrome Screens and Processes of Making the Same; and we do hereby declare the following to be a full, clear, and exact description of the invention, such as will enable others skilled in the art to which it appertains to make and use the same.

Our invention relates to polychrome screens for color photography.

For making photographic pictures in natural colors by the trichromatic process three layers dyed in the three primary colors are necessary which are used at first as receiving filters, either as complete layers or in the form of screens, and afterward for producing the colored picture.

In color screens such as are now in use the receiving filters or color screen elements are used for producing the colored picture. But when making therefrom colored paper pictures it is absolutely necessary, that the colored elements which produce the pictures have a considerably lighter tint and are much more translucent than before when serving as receiving filters.

By means of the color screens which have heretofore been in use a good paper picture can not be produced, because the filter elements must be so strongly dyed, and are therefore so deeply colored that they can not be used thereafter as elements for producing the picture.

The object of the improvements is to avoid this objection. And with this object in view our invention consists in providing a color screen which has a lighter tint when producing the picture than before, when it acted as a filter. As a foundation a screen plate is used which is made for example from suitable screen materials as from colloidal substances such as gelatin. A solution of gelatin is dyed with two dye stuffs of the same color (not necessarily of the same depth of color) but different properties and atomized in a suitably heated chamber; by choosing an appropriate height of fall the size of the resultant colored particles may be determined. This operation is carried out, for a given screen, with each of the three primary

colors. Thereby two kinds of dyestuffs are applied to each color screen, one of which is fixed or can be fixed in the colloid forming the foundation, while the other one can afterward easily be removed. This may be done for example by washing the same out, in which case dyestuffs of acid and basic character are used, for the reason that, as is known in the art, the acid dyestuff can not be removed from the gelatin by washing, while the dyestuffs of basic character can easily be washed out. The color screen which has thus been prepared is used in the following way after first applying a sensitive emulsion: The color screen is exposed to the light from the rear and through the filtering elements and developed in the usual way. After fixing and washing a sheet of paper is pressed thereon and the whole layer is drawn off, so that the filtering elements are brought to the top. In case of colloids which are soluble in water, such as gelatin or starch, the layer is drawn off according to methods known in photomechanics. For example, the plate is brought into a diluted solution of hydrofluoric acid (1%), whereby gas globules of silicon tetrafluorid are formed on the glass which permit the layer to float off (see Eder, *Rezept u. Tab.*, page 30). Or the glass plates are coated with an exceedingly thin layer of caoutchouc and collodion. When using resin as screen layers the glass plates are treated with talcum. After the picture has been drawn off it is washed until the non-fixed dyestuffs have completely been removed.

As an example, the following dyestuffs will be given, which are suitable for colloids containing water, such for example as starch: For each screen we use one mordant dyestuff, such for example as fuchsin, malachite green, patent blue, otherwise known as the disulfonic acid of the condensation product from metaoxybenzaldehyde, and one acid dyestuff, such for example as oxamin red, oxamin green, and oxamin blue. The mordant dyestuffs are fixed by potassiumantimonyltartrate and tannin, while the acid dyestuffs remain soluble and can be washed out. When carrying this method out for each screen 100 grams of starch are dyed; in one case with fuchsin 5 grams, oxamin red 5 grams, in the second case with malachite green 5 grams, oxamin green 5 grams, and in the 110

third case with patent blue 5 grams, oxamin blue 5 grams.

For resin screens dyestuffs may be used for example which are soluble in petroleum 5 benzin, for example Sudan III agfa, Sudan IV agfa, moti-yellow Weiler ter mer, moti-blue Weiler ter mer, and others which are not soluble in petroleum benzin, such for example as fuchsin Höchst, naphthalene yellow Casella; spirit blue Casella otherwise known as chlorhydrate (sulfate or acetate) of triphenyl-p-rosenalin and triphenyl rosenalin (see Dammer *Chemische Technologie der Neuzeit* 1911, Vol. II page 980). The following example gives good results: For each plate 100 grams of mastix resin are dyed in one case with Sudan III agfa 5 grams, fuchsin Höchst 5 grams, in the second case with moti-yellow Weiler ter mer 5 grams, naphthalene yellow Casella 5 grams, in the third case with moti-blue Weiler t. m. 5 grams, spirit-blue Casella 5 grams. From these three masses of resin which have been dyed with different dyestuffs a single screen is made in the usual way which after the picture has been completed are treated with benzin, so that the soluble dyestuff is removed. Furthermore we may use dyestuffs which are adapted to be bleached by light together with such dyestuffs which are not bleached. For example Fulpid dyestuffs may be used which have been described in Eder, *Jahrbuch* 1910, page 161. The screens are afterward exposed to the light, so that one of the dyestuffs is bleached out. As the time which is required for affecting the silver bromid element is short as compared to the time which is necessary for changing the Fulpid dyestuffs, the latter are not destroyed while the picture is being taken.

The following is an example of the use of Fulpid dyestuffs with colloids containing water: In each case 100 grams of colloid are dyed in one case with fuchsin Höchst 5 grams, Fulpid red 5 grams, in the second case with auramin Höchst 5 grams, Fulpid yellow 5 grams, in the third case with Victoria blue Höchst 5 grams, dicyanin Höchst 5 grams.

Each screen is made in the manner described above and then sensitized, and it is exposed after development to the free sun light about one minute, or to the diffused day light or electric arc light, etc., about 10 or 15 minutes. Thereby the Fulpid dye-

stuffs and dicyanin are bleached out, while the other dyestuffs are not altered.

An example for resin screens is the following: In each case 100 grams of colophony are dyed in one case with Sudan IV agfa 5 grams, Fulpid red 5 grams; in the second case with naphthalene yellow 5 grams, Fulpid yellow 5 grams, in the third case with spirit blue Casella 5 grams, dicyanin Höchst 5 grams.

In the present case the picture forms no part of the invention claimed, which invention comprises only the screen prepared with its two kinds of dyestuffs one fixed and the other removable, in the three primary colors.

We claim herein as our invention:

1. In the process of making a polychrome screen the step which comprises treating a suitable screen material with two coloring materials of the same tint, the tint of one of said materials being fixed and of the other removable, and applying said colored screen material to a suitable light penetrative support.

2. In the process of making a polychrome screen the step which comprises treating a colloid screen material with two coloring materials of the same tint, the tint of one of said materials being fixed and of the other removable, and applying said colored screen material to a suitable light penetrative support.

3. In the process of making a polychrome screen the step which comprises treating gelatin screen material with two coloring materials of the same tint, the tint of one of said materials being fixed and of the other removable, and applying said colored gelatin to a suitable light penetrative support.

4. A polychrome screen comprising a suitable light penetrative support and a layer of screen material upon said support said material being colored with two different coloring materials of the same tint in each of the three primary colors the tint due to one of said materials being fixed and that due to the other of said materials being removable.

In testimony whereof we hereunto affix our signatures in the presence of two witnesses.

RUDOLF RUTH.  
ALADAR SCHULLER.

Witnesses:

E. JACOBS,  
N. ADAMS.